

# UNITED STATES PATENT OFFICE.

LAWRENCE ADDICKS, OF DOUGLAS, ARIZONA.

## PROCESS OF RECOVERING METALS BY ELECTROLYSIS.

1,138,921.

Specification of Letters Patent.

Patented May 11, 1915.

No Drawing.

Application filed November 5, 1914. Serial No. 870,440.

*To all whom it may concern:*

Be it known that I, LAWRENCE ADDICKS, a citizen of the United States of America, residing in Douglas, in the county of Cochise and State of Arizona, have invented certain new and useful Improvements in Processes of Recovering Metals by Electrolysis, of which the following is a specification.

10 This invention relates to a process of electrolysis, more especially to the electrolysis of copper, and aims to provide improvements therein.

15 In the electrolysis of metals, and in particular copper, the presence of certain compounds of metals other than that to be deposited, occurring in the electrolyte or formed therein by the reaction occurring during the electrolysis, exercises a solvent 20 action on the deposited metal, which is often detrimental. For instance, copper ores usually contain iron, and when the copper ore is dissolved, iron compounds are also dissolved, and are mixed with the copper compounds 25 in the liquid. Or, iron compounds may be introduced in the electrolyte for the purpose of depolarizing. When these iron compounds are in the -ous state they will be oxidized to the -ic state by the action occurring at the anode. Ferric compounds are reduced by copper, and consequently the ferric compounds occurring in 30 the electrolyte would act to dissolve the deposited copper.

35 Ferric salts have in fact long been known as active oxidizing agents applicable to the lixiviation of the mineral values in certain ores. Well-known processes, such as that commonly known as the Siemens-Halske, 40 have been evolved where ferrous sulfate is converted into ferric sulfate by anodic oxidation in an electrolytic cell, the corresponding cathodic reduction being used to deposit copper in this case, the depleted and oxidized electrolyte being returned to the lixiviation tanks, thereby making the process 45 cyclical. The ferrous sulfate at the same time acts as a depolarizer in the cell, the equivalent of the chemical energy of anodic 50 oxidation appearing as a corresponding lowering of voltage under proper conditions of operation.

55 The great difficulty in such processes is in keeping the ferric sulfate formed from attacking and redissolving the cathodes there-by wholly or in part making the useful

yield of the cell too low for commercial purposes. Two methods have been proposed to overcome this (a) the use of a mechanical diaphragm to keep the anolyte and catholyte 60 separate; and (b) the injection of sulfur dioxide gas into the cell which is in effect a chemical diaphragm in that it reduces the ferric salt to the ferrous salt, at the same time being itself oxidized to sulfuric acid; 65 it also partly displaces the ferrous salt as a depolarizer, being itself oxidized to sulfuric acid directly at the anode. The first plan is open to many mechanical and electrical objections and has not found general favor. 70 The second vitiates the atmosphere of the cell room, is limited to an ore which can be economically leached by sulfuric acid, and requires a somewhat prodigal use of sulfur dioxide in order to attain the desired result. 75

I have found that the activity of the metal compounds which exercise a solvent action on the metal being deposited depends upon (a) the concentration of the compound in the solution; (b) the temperature of the 80 solution; (c) the time of exposure of the deposited metal to attack; (d) the surface of the deposited metal exposed, and (e) the concentration of other salts in the solution.

It is evident that within certain limits, 85 (a), (b), (c), and (d) can be favorably balanced by the choice of a suitable rate of circulation through the cell, current density, etc., but (e) is the controlling factor.

In general the presence in quantity of a 90 compound or compounds other than that of the metal to be deposited in such an electrolyte as referred to, that is, one containing a compound of the metal to be deposited and a compound exercising a solvent action on the deposited metal, seems to have a deterrent effect on the activity of the solvent compound, this being very markedly so in the case of aluminum sulfate. I therefore use in a cell, a sulfate copper electrolyte for example, with sufficient cupric sulfate and ferrous sulfate present to give a good deposit of copper at the cathode and efficient depolarization at the anode (anodic oxidation) for the circulation used. I also use 95 sufficient aluminum sulfate to retard the corrosion rate at the cathode to a small proportion of the quantity of copper deposited per unit of time at the current density used, and yet not so much aluminum sulfate as to 100 practically inhibit this activity which would render very difficult the reduction of the

ferric sulfate by other means when it is desired to utilize, outside of the cell, the solution containing the ferric sulfate. As a practical illustration I find a suitable set of 5 conditions for good work to be, using a carbon anode and copper cathode, a solution containing copper, iron and aluminum salts, all as sulfates, showing on analysis 3% copper, 3% ferrous iron and 3% alumina, some 10 free sulfuric acid to prevent the formation of basic salts, a current density of 13.5 amperes per sq. ft., a temperature of 115° F. and a circulation sufficient to hold the average concentration of ferric iron present to 15 about 0.25%. Under such conditions a cathode deposit equivalent to from 70% to 90% of the theoretical can be obtained.

After leaving the cells the solution can be used direct upon ores containing native 20 copper such as the tailings dumps in Michigan, which carry lake "mineral," or for extracting the finely divided copper contained in anode slimes from copper refining preparatory to their treatment for the 25 recovery of silver and gold by well known processes. In these cases the lessened activity of the reaction due to the presence of aluminum and other sulfates is compensated for by the great surface exposed by 30 the fine state of sub-division in which the copper exists. The reduction is thorough and 90% current efficiency should be obtained.

Certain sulfid ores may also be attacked 35 directly, but it is generally advisable to give these a preliminary roast, thereby transferring them to the oxidized class.

In the case of oxid ores, the ferric sulfate may be reduced by suitable means such 40 as sulfur dioxide gas, resulting in the formation of sulfuric acid which is used as the leaching agent for oxids, silicate and carbonates of copper, the sulfate being directly soluble in water. Theoretically a free 45 acid yield of about three pounds per lb. of copper deposited can be obtained in this way, half being supplied by the ferric sulfate reduced and half by the sulfuric acid oxidized. When the gas is weak in  $\text{SO}_2$ , 50 owing to its being a by-product from roasting, it may be difficult to obtain complete reduction so that some iron sulfate enters the cell unreduced making it difficult to keep the average ferric iron in the cell down to the 55 desired point, resulting in an undesirably low current efficiency. In such cases a certain proportion of the copper leached may be cemented upon iron, the electrolyte leaving the cells first being subjected to the action 60 of the  $\text{SO}_2$  and then to that of the cement copper. This will properly reduce the solution and restore the cell efficiency. Cementation at the same time affords a means of lowering the electrolyte in salts. The 65 composition of the electrolyte must be main-

tained in any case by systematic additions and withdrawals, the ore generally furnishing the desired source of alumina and iron, as well as of copper.

What is claimed is:—

1. In a process for the electrolytic reduction of metals in the presence of a substance having a solvent action upon the deposited metal, electrolyzing in the presence of a salt adapted to counteract the solvent action of 70 said substance having the dissolving action.

2. In a process for the electrolytic reduction of metals in the presence of a substance having a solvent action upon the deposited metal, electrolyzing in the presence of a sulfate adapted to counteract the solvent action of 80 said substance having the dissolving action.

3. In a process for the electrolytic reduction of metals in the presence of a substance 85 having a solvent action upon the deposited metal, electrolyzing in the presence of aluminum sulfate of a concentration adapted to counteract the solvent action of said substance having the dissolving action.

4. In a process for the electrolytic reduction of metals in the presence of a substance having a solvent action upon the deposited metal, electrolyzing in the presence of a substance adapted to counteract the solvent action 90 of said substance having the dissolving action, said counteracting substance being present in amount sufficient to materially reduce the degree of attack on the cathode and yet insufficient to deaden its effect, 100 whereby the solution may be sufficiently used as a solvent for metals or ores.

5. In a process for the electrolytic reduction of copper in the presence of a depolarizer which acts to form a substance 105 having a solvent action upon the deposited copper, electrolyzing in the presence of a salt adapted to counteract the solvent action of said substance having the dissolving action.

6. In a process for the electrolytic reduction of copper in the presence of an iron salt having a solvent action upon the deposited copper, electrolyzing in the presence of a salt adapted to counteract the solvent 115 action of the iron salt.

7. In a process for the electrolytic reduction of copper in the presence of an iron salt having a solvent action upon the deposited copper, electrolyzing in the presence 120 of aluminum sulfate of a concentration adapted to counteract the solvent action of said iron salt.

8. In a process for the electrolytic reduction of copper in the presence of an iron 125 salt having a solvent action upon the deposited copper, electrolyzing in the presence of aluminum sulfate adapted to counteract the solvent action of said iron salt, said aluminum sulfate being present in amount 130

sufficient to materially reduce the degree of attack on the cathode and yet insufficient to deaden the leaching effect of the solution.

9. In a process for the electrolytic reduction of copper, electrolyzing in the presence of a ferrous compound adapted to operate as a depolarizer, and in the presence of a substance adapted to counteract the solvent action of the ferric compound formed in the electrolyte.

10. In a process for the electrolytic reduction of copper, electrolyzing in the presence of a ferrous salt adapted to operate as a depolarizer, and in the presence of a substance adapted to counteract the solvent action of the ferric salt formed in the electrolyte.

11. In a process for the electrolytic reduction of copper, electrolyzing in the presence of a ferrous salt adapted to operate as a depolarizer, and in the presence of a salt adapted to counteract the solvent action of the ferric salt formed in the electrolyte.

12. In a process for the electrolytic reduction of copper, electrolyzing in the presence of a ferrous salt adapted to operate as a depolarizer, and in the presence of aluminum sulfate of a concentration adapted to counteract the solvent action of the ferric salt formed in the electrolyte.

13. In a process for the electrolytic reduction of copper, electrolyzing in the presence of a ferrous salt adapted to operate as a depolarizer, and in the presence of a substance adapted to counteract the solvent action of the ferric salt formed in the electrolyte, said counteracting salt being present in amount sufficient to materially reduce the degree of attack on the cathode and yet insufficient to deaden the leaching effect of the solution.

14. In a process for the electrolytic reduction of metals in the presence of a substance

having a solvent action upon the deposited metal, electrolyzing in the presence of a substance adapted to counteract the solvent action of said substance having the dissolving action, and using portions from the bath for the dissolving of metal compounds to be electrolyzed.

15. In a process for the electrolytic reduction of copper in the presence of a salt having a solvent action upon the deposited copper, electrolyzing in the presence of a salt adapted to counteract the solvent action of said salt having the dissolving action, and using portions from the bath for the dissolving of metal compounds to be electrolyzed.

16. In a process for the electrolytic reduction of copper, electrolyzing in the presence of a ferrous salt adapted to operate as a depolarizer, and in the presence of a substance adapted to counteract the solvent action of the ferric salt formed in the electrolyte, and using portions from the bath for the dissolving of copper compounds to be electrolyzed.

17. In a process for the electrolytic reduction of copper, electrolyzing in the presence of a ferrous salt adapted to operate as a depolarizer, and in the presence of aluminum sulfate of a concentration adapted to counteract the solvent action of the ferric salt formed in the electrolyte, and using portions from the bath for the dissolving of copper compounds to be electrolyzed.

In witness whereof, I have hereunto signed my name in the presence of two subscribing witnesses.

LAWRENCE ADDICKS.

Witnesses:

GEORGE FORDHAM,  
KATHERINE CONKLIN.